

**1**

3,421,987

**ELECTROCHEMICAL MACHINING USING A FILM FORMING ELECTROLYTE INCLUDING AMINE ALCOHOLS**

Mitchell A. La Boda, East Detroit, Mich., assignor to General Motors Corporation, Detroit, Mich., a corporation of Delaware

No Drawing. Filed Oct. 23, 1965, Ser. No. 504,108  
U.S. Cl. 204—143  
Int. Cl. B23p 1/16

3 Claims

**ABSTRACT OF THE DISCLOSURE**

Electrochemical erosion-inhibiting film-forming electrolytes for electrochemically machining ferrous metals, consisting essentially of aqueous solutions of alkali metal chlorides and amines of low molecular weight alcohols.

This invention relates to electrochemical machining processes and, more particularly, to electrolytes for use therewith.

In recent years electrolytic machining procedures for generating shapes, cavities and contoured surfaces have been developed and are more generally classified into one of two basic categories, the first being electrochemical machining and the second electrolytic grinding, a specialized application of the first. Electrolytic grinding is essentially an electrochemical deplating process which can be used on virtually any electrically conductive material. It is generally adapted to metal removal operations comparable to those performed by cutoff wheels, saws, and grinding or milling machines and the like, and uses equipment similar to conventional grinders except for the electrical accessories. About 95% of the metal removal results from electrolytic rather than mechanical action.

A particular version of an electrolytic grinding process is characterized by a flow of electrolyte between the workpiece and a rotating grinding cathode wheel. The rotating cathode wheel comprises a conductive metal matrix having a plurality of nonconducting abrasive particles imbedded therein to provide nonconductive spacing between the workpiece and the cathodic matrix. Electric current is passed through the electrolyte to dissolve the anodic surfaces of the workpiece and the imbedded particles of the wheel abrade the surface to remove any irregularities resulting from nonuniform erosion or reaction product build-up.

While aqueous solutions of individual inorganic salts, such as nitrates, cyanides, carbonates, hydroxides and nitrites have been used as electrolytes in electrochemical machining and grinding processes, none has offered any significant advantage over the now well accepted aqueous sodium chloride solution most commonly used today. However, regardless of what salt is chosen, an apparent problem with electrochemical machining and grinding processes using that salt singularly or in combination is overcut, which is the uncontrolled anodic dissolution of the workpiece in unwanted areas resulting in undesirable tapering of holes, rounding of edges, and the like. Such anodic dissolution can occur in areas which are fairly well removed from the cathode. This overcut, or cutting in low current density areas which are bathed in the electrolyte but substantially removed from the cathode, has been substantially reduced in the prior art by the use of costly and time-consuming masking operations which isolate the areas to be machined by protecting the surrounding areas from the erosive effect of the electrolyte. These masking operations are frequently quite involved and require a high degree of skill to insure a satisfactory product. Likewise, additional steps subsequent to the machining steps are required to strip the workpiece of the mask. Additionally,

**2**

the prior art has attempted to reduce overcut by designing special purpose electrodes and machines to meet individual and specialized machining requirements.

By my invention I have at least reduced, and in most cases actually eliminated, the need for recourse to the prior art's attempted resolutions.

It is, therefore, an object of my invention to provide a self-masking electrolyte for ECM.

It is a further object of my invention to provide an additive for existing ECM electrolytes which inhibits anodic dissolution.

It is a further object of my invention to effect a sharply contoured machining by a process utilizing a basic aqueous electrolyte containing known salts and improving same by adding thereto a compound which upon reaction with the workpiece forms a film thereover, which film inhibits or stops off electrolytic action or anodic dissolution, and subsequently removing said film in selected areas to permit continued machining exclusively in those areas.

It is a further object of my invention to effect a sharply contoured electrochemical machining by a process utilizing aqueous electrolytes containing known salts and an additive consisting of an amine of a low molecular weight alcohol, particularly primary, secondary and tertiary ethanolamine.

Further objects and advantages of the present invention will become apparent from the following detailed description of the invention.

My invention briefly stated involves adding an amine of a low molecular weight alcohol to substantially neutral ECM electrolytes. By an amine of a low molecular weight alcohol, I mean up to and including the butanolamines. When added to ECM electrolytes the additives of my invention, and especially the ethanolamines, create a solution which effectively forms a heavy adherent film over the surface of the workpiece. The film retards or substantially eliminates electrochemical erosion in those areas protected by the film. In a particular application a chloride electrolytic grinding electrolyte is modified in accordance with my invention. The film formed is subsequently abraded away in those areas where electrochemical machining is to continue, hence presenting a limited uninhibited surface to unrestricted electrochemical action.

My experience has been that using the additives of my invention, I can successfully machine metal samples ranging from the softer low carbon steels (SAE 1008) to the harder low alloy steels (SAE 5160H). However, the additive of my invention will be likewise applicable and effective for ferrous alloys wherein the iron content is 50% or more.

While the preferred electrolytes comprise either about 4.3 to 18.43% by weight of monoethanolamine or about 3.4 to 9.1% by weight of triethanolamine or combinations thereof, I have found that effective electrolytes can be compounded using from 2.2 to 42.0% by weight of ethanolamine, the balance being a selected concentration of an aqueous sodium chloride solution wherein the concentration of the sodium chloride may vary from dilute to saturated. In this connection the lighter alkali metal (lithium, sodium and potassium) chlorides are preferred because they produce relatively neutral pH's, do not plate out or have a deleterious effect upon the cathode, and represent a source of inexpensive material. Likewise, while electrolytes dilute as to chloride ion are operative, as a practical matter there are no significant advantages to operating at the lower concentrations and, in fact, it is less desirable to do so when considering such factors as solution conductivity and the like. Hence solutions in the order of 15-20% NaCl are preferred.

While there is every indication that the soluble higher aliphatic alcohol amines, i.e. pentanolamine and above,

will be equally operative, their availability and cost have rendered their use impractical.

I have been successful in operating these electrolytes at voltages up to 40 volts and anode current densities from 5 to 500 amperes per square inch. However, for each particular additive concentration there appeared to be a maximum current density above which practical control over the machining was lost.

The exact explanation for this was not ascertained, but

Tube length decrease per unit time was used to determine metal removal rates. The tube ends were compared with those produced by electro-chemically grinding similar samples under the same conditions with additive-free electrolytes. Similar tests were conducted with non-tubular stock material.

The following table represents the results of experiments conducted in accordance with the procedure outlined above.

TABLE

| Additive | Conc. (mls.) (1) | Volts (v.) | Current density (a.s.i.) | Metal removal rate, in./min. | Sample SAE | Results                                               |
|----------|------------------|------------|--------------------------|------------------------------|------------|-------------------------------------------------------|
| MEA----- | 25               | 3.8        | 290                      | 0.029                        | 1018       | Very square cut. Little burr left.                    |
| MEA----- | 25               | 8.4        | 540                      | 0.063                        | 1018       | Some loss of corner; little burr on trailing side.    |
| MEA----- | 50               | 4.0        | 250-290                  | 0.026                        | 1018       | Slight evidence of inhib.                             |
| MEA----- | 50               | 8.5        | 540                      | 0.064                        | 1018       | Slight evidence of inhib.                             |
| MEA----- | 200              | 4.0        | 290                      | 0.008                        | 1018       | ECM stopped. Mechanical component 0.008.              |
| MEA----- | 200              | 4.0        | 260                      | 0.001                        | 1018       | ECM stopped.                                          |
| MEA----- | 200              | 4.5        | 115-155                  | 0.011                        | 1018       | ECM stopped.                                          |
| MEA----- | 200              | 9.5        | 230                      | 0.027                        | 1018       | ECM slowed to fraction of NaCl solution.              |
| TEA----- | 25               | 4.1        | 230                      | 0.034                        | 1018       | Inhib. Indef.                                         |
| TEA----- | 25               | -----      | -----                    | 0.011                        | 1018       | Mechanical cutting component.                         |
| TEA----- | 25               | 8.7        | 460                      | 0.066                        | 1018       | No inhib.                                             |
| TEA----- | 50               | 4.2        | 250                      | 0.032                        | 1018       | Strong inhib. Little burr left.                       |
| TEA----- | 50               | 8.7        | 460                      | 0.066                        | 1018       | Too little inhib. at this current density.            |
| TEA----- | 100              | 4.2        | 250                      | 0.026                        | 1018       | Front inhib. increased; side inhib. good.             |
| TEA----- | 100              | 8.8        | 425                      | 0.058                        | 1018       | Front inhib. increased; side inhib. good.             |
| MEA----- | 100              | 4.5        | 100                      | 0.012                        | 5160H      | Strong inhib.                                         |
| MEA----- | 100              | 9.2        | 260                      | 0.028                        | 5160H      | Insufficient inhib. at this current density.          |
| MEA----- | 100              | 4.3        | 80-100                   | 0.010                        | 4620       | Inhib., but not strong.                               |
| MEA----- | 100              | 9.3        | 260-285                  | 0.025                        | 4620       | Inhib., but not strong.                               |
| MEA----- | 200              | 4.5        | 75-100                   | 0.008                        | 5160H      | Strong inhib., poor surface finish.                   |
| MEA----- | 200              | 4.5        | 75                       | 0.005                        | 4620       | Strong inhib., poor surface finish.                   |
| MEA----- | 250              | 4.8        | 75                       | 0.007                        | 5160H      | Strong inhib.; finish improved.                       |
| MEA----- | 250              | 4.8        | 75                       | 0.005                        | 4620       | Strong inhib.; finish improved.                       |
| MEA----- | 300              | 4.7        | 75                       | 0.006                        | 5160H      | Excellent inhib.; surface finish improved.            |
| MEA----- | 300              | 4.7        | 50-75                    | 0.004                        | 4620       | Very good inhib.; finish improving.                   |
| MEA----- | 400              | 4.7        | 40                       | 0.0035                       | 5160H      | Excellent inhib.; excellent finish.                   |
| MEA----- | 400              | 9.75       | 130                      | 0.013                        | 5160H      | Excellent inhib.; excellent finish.                   |
| MEA----- | 400              | 4.5        | 25                       | 0.003                        | 4620       | Very good inhib.; good finish.                        |
| MEA----- | 400              | 9.5        | 115                      | 0.011                        | 4620       | Very good inhib. and finish.                          |
| MEA----- | 400              | 15.2       | 230                      | 0.019                        | 4620       | Very strong inhib.; good surface finish.              |
| MEA----- | 500              | 4.6        | 17                       | 0.0025                       | 5160H      | Perfect inhib.; ECM stopped.                          |
| MEA----- | 500              | 9.8        | 120                      | 0.011                        | 5160H      | Excellent tip. Excellent inhib. and finish.           |
| MEA----- | 500              | 15.2       | 190                      | 0.017                        | 5160H      | Very good tip; good inhib. and finish.                |
| MEA----- | 500              | 4.7        | 12                       | 0.004                        | 4620       | Perfect inhib.; acceptable finish.                    |
| MEA----- | 500              | 9.8        | 100-130                  | 0.010                        | 4620       | Excellent tip; unsat. finish.                         |
| MEA----- | 500              | 15.2       | 230                      | 0.016                        | 4620       | Excellent inhib.; good finish.                        |
| MEA----- | 600              | 4.7        | 17-25                    | 0.005                        | 5160H      | Very good tip; strong inhib.; good finish.            |
| MEA----- | 600              | 9.8        | 90-100                   | 0.009                        | 5160H      | Very good inhib. and finish.                          |
| MEA----- | 600              | 15.2       | 190                      | 0.018                        | 5160H      | Excellent tip, inhib. and finish.                     |
| MEA----- | 600              | 20.1       | 260                      | 0.020                        | 5160H      | Unsat. inhib. and finish—best at this voltage.        |
| MEA----- | 600              | 4.7        | 17                       | 0.002                        | 4620       | Good inhib. and finish.                               |
| MEA----- | 600              | 9.8        | 90-100                   | 0.0075                       | 4620       | Good tip, inhib. and finish.                          |
| MEA----- | 800              | 4.7        | 4-8                      | 0.003                        | 5160H      | Very strong inhib., ECM about stopped.                |
| MEA----- | 800              | 9.8        | 63                       | 0.0007                       | 5160H      | Very good inhib. and finish.                          |
| MEA----- | 800              | 9.8        | 63-100                   | 0.009                        | 5160H      | Very good inhib.                                      |
| MEA----- | 800              | 4.7        | 10                       | 0.003                        | 4620       | Very good tip—not improved over lower concentrations. |
| MEA----- | 800              | 9.8        | 100-125                  | 0.0085                       | 4620       | Very good inhib.                                      |
| TPA----- | 50               | 4.0        | 50                       | 0.010                        | 5160H      | Fair inhib. and finish.                               |
| TPA----- | 50               | 9.0        | 300                      | 0.030                        | 5160H      | Inhib. improved over lower current density samples.   |

<sup>1</sup> Mls. of amino alcohol added to 1 liter 18% NaCl solution.

MEA=Monoethanolamine, TEA=Triethanolamine, TPA=Triisopropanolamine (mix).

it is felt that the film formed may be breaking down at the higher current densities, much like has been disclosed in my copending patent application Ser. No. 504,133, filed Oct. 23, 1965.

Generally speaking, tests were conducted utilizing a system wherein steel tube samples were brought up to a rotating sintered bronze diamond impregnated wheel. A gravity feed system kept the samples at the face of the wheel at all times. The feed system was such that an adjustable weight provided the capability of varying the pressures at which the samples would engage the wheel. It was found that to properly evaluate the inhibitive effects of my additives a minimum workpiece-to-wheel pressure should be employed in order to reduce the mechanical cutting component of the abrasive wheel. A room temperature electrolyte was pumped at a pressure of 9 p.s.i. through a bore in the workpiece and into the gap between the cathode and the workpiece at a rate of 0.25 gallon per minute. This gap was held constant by the spacer effect of the nonconductive diamond chips.

Other than abrasive means for the local removal of the inhibiting film of my invention may be employed. Among the possibilities might be localized breakdown under high current densities, localized flushing, and/or a variety of sophisticated variations of these and others. Therefore, though my invention has been described in terms of certain preferred embodiments, it is to be understood that others may be adapted and that the scope of my invention is not limited except by the appended claims.

I claim:

1. A process for electrochemically machining a ferrous metal comprising the steps of establishing said metal as the anode in an electrochemical cell, orienting a cathode electrode adjacent to but closely spaced from said metal so as to form a gap therebetween, flowing through said gap a substantially neutral electrolyte consisting essentially of an aqueous solution of at least one alkali metal chloride and at least one amine of a low molecular weight alcohol in concentrations of from about 2.2 percent by weight to about 42.0 percent by weight to form an elec-

trochemical erosion inhibiting film on said metal, passing current through said cell and removing from selected areas the electrochemical erosion inhibiting film formed whereby electrochemical machining can continue in said areas.

2. The process as claimed in claim 1 wherein said alcohol is ethanolamine having a concentration of from about 2.2 to about 42.0% by weight.

3. The process as claimed in claim 2 wherein the concentration of said ethanolamine is 3.4 to 18.4% by weight.

## References Cited

## UNITED STATES PATENTS

2,939,825 6/1960 Faust, et al. ----- 204—142

ROBERT K. MICHALEK, *Primary Examiner.*

U.S. Cl. X.R.

252—79.4